

## UNITED STATES PATENT OFFICE

DE VERE DIERKS, OF KANSAS CITY, MISSOURI

## PROCESS OF TREATING LUMBER

No Drawing.

Application filed June 28, 1927. Serial No. 202,168.

This invention relates to the manufacture of lumber and is concerned more particularly with the production of dressed lumber which is supplied to the trade for numerous purposes, such as flooring, interior trim, and the like, and is also used in the manufacture of various articles.

Dressed lumber is now produced from rough dimension stock which is dried, ordinarily in kilns, to a selected moisture content, then surfaced by planers and sometimes given a beading, or worked into mouldings and other special forms. Upon the completion of the dressing operations, the finished product is usually shipped without delay for use, but as it is exposed to varying atmospheric conditions during shipment and also in actual use, the moisture content frequently changes, causing the lumber to shrink or swell as moisture is lost or taken up. Change in moisture content also results in checking, cracking, warping, etc., and any shipment consequently is liable to reach its destination with a percentage of lumber falling below specification and therefore rejected as unfit for use, or else accepted as of an inferior quality. Such lumber not only represents an actual loss to the manufacturer in lower return, but also frequently results in claims for damage, so that changes in the lumber due to variation in the moisture content present a serious problem. Similarly, the occurrence of defects in the dressed lumber while in use, such as shrinking, swelling, etc., causes trouble to the ultimate consumer and likewise injures the reputation of the manufacturer, even though these defects arise from no fault in manufacture.

These difficulties cannot be overcome by improvements or alteration in the method of drying the rough stock, since they do not occur because of imperfect or insufficient drying, but because of changes in the moisture content after the drying and dressing operations have been completed, and may be the result of loss of moisture, as well as of absorption.

In order to avoid these defects in the dressed product, I have devised a method of producing dressed lumber which retains its

original moisture content for an indefinite period, or under severe conditions, changes in moisture content only at a relatively low rate. To accomplish this end I seal the lumber immediately upon the completion of the drying operations, and for this purpose I apply to the wood a sealing material or coating which is substantially waterproof or impervious to moisture. This material forms a thin, clear, hard, surface film which closes and seals the pores of the wood and also permeates the wood to a substantial extent. The sealing material in no way interferes with the use of the lumber, but in addition to the primary function of sealing the pores of the wood, it effects a substantial economy on behalf of the ultimate consumer in that the sealing film serves as a priming coat and thus reduces the number of coats of finish ordinarily required.

According to my invention, the sealing material is applied to the lumber immediately after the latter has been dressed in appropriate machines. For this purpose, the finished product is carried from the finishing machines directly into a bath of the sealing material, a conveyor being preferably employed for the purpose which receives the lumber from the dressing machines and carries it into, through, and out of a tank in which it is immersed in the sealing material by a simple dipping operation. The lumber is then allowed to dry and the drying may be hastened by forced draft, if desired. After the surface is dry, the lumber may be shipped and each piece is coated with a thin, hard layer of the colorless sealing compound which imparts a slight sheen or gloss to a plane surface, and also darkens the wood to a very slight extent, so that the grain stands out more prominently. The lumber so treated is not subject to ordinary defects, such as variation in dimension, distortion, checking, cupping, etc., and thus is of superior quality and may be sold at a higher market price.

While it is generally satisfactory to apply the sealing material to the dressed lumber immediately upon the completion of the dressing operations, the best results may be obtained by reducing to a minimum the length

of time that the lumber is exposed to the atmosphere after it leaves the kiln and before it is coated with the sealing material. At the end of the drying operation, the lumber taken from the kiln contains a selected amount of moisture, as, for example 7 or 8%, this content being determined by the manner in which the drying operation is carried out in the kiln. This kiln-dried lumber should then be dressed 10 with a minimum of delay and immediately after being finished and shaped to proper form, the dressed product should be sealed so that in the final product carrying a sealing coating on all its exterior surfaces there is 15 present substantially the same amount of moisture present in the wood as it is taken from the kiln.

The solution which I prefer to use for the sealing treatment includes a number of 20 ingredients which are selected to produce a mixture of waterproofing quality and high penetrating power, this solution drying quickly so as to provide a hard, clear coating. In order to secure the necessary waterproofing qualities, China wood or tung oil 25 is employed, this oil being first treated to make it capable of providing a waterproofing layer, according to any of the usual methods commonly employed for this purpose by 30 varnish manufacturers. China wood oil thus treated is highly satisfactory for the purpose, since it dries hard and clear.

To the treated China wood oil is added a quantity of a suitable compound which 35 will give the mixture the desired penetrating power, and for this purpose xylol may be used. Xylol is a constituent of coal tar naphtha well known among varnish manufacturers and it has the quality of penetrating 40 the pores of wood, it dries rapidly, and it does not leave a greasy spot. Other compounds may be used to replace xylol, as, for example, so-called "solvent naphtha" or toluol, although xylol appears to be the most 45 satisfactory. The desired material is one which penetrates rapidly, minglest freely with China wood oil, dries quickly, and does not stain. The proportions in which the waterproofing material and the penetrating material 50 are employed in the mixture will vary somewhat according to whether the qualities of waterproofing or penetrating are to predominate. Likewise, the type of penetrating material to be used may depend on the 55 rate of drying desired. Commercial "solvent naphtha" evaporates somewhat more slowly than xylol, while toluol evaporates somewhat more rapidly.

A solution for ordinary use may be made 60 up of 50% treated China wood oil and 50% xylol. To the China wood oil may be added a small amount of a suitable dryer, such as a cobalt dryer. Also, if desired, a pigment 65 may be added to the mixture, this pigment assisting to close the pores of the wood

and giving the surface a slight roughness so that finishing materials will adhere better. As a suitable pigment, numerous materials may be employed, such as a mixture of asbestos (magnesium silicate) 75%, 70 china clay (aluminum silicate) 20%, and bentonite clay 5%. This pigment may be used in varying amounts with the mixture of China wood oil and the penetrating medium above described, as, for example, there 75 may be mixed with the solution an amount of pigment equal to 20% of the total weight of the mixture. The pigment is prepared in the ordinary manner and is ground fine for use. 80

In carrying out the novel treatment, the rough stock dried to a selected moisture content, for example 8%, is sawed, planed, beaded, etc., in accordance with the standard practice to produce the desired product. The dressed lumber is then taken directly from the machines and dipped in the solution tanks, the lumber travelling through the tanks at a suitable rate of speed so that 85 it is immersed for one or two minutes. During this immersion, the China wood oil is carried into the pores of the wood by the penetrating medium to a substantial extent. Beyond the tanks the lumber is moved along slowly, so that the surface coating may dry 90 to an extent sufficient to prevent tackiness and after the surface of the lumber has dried, it may be stacked or handled in the usual way, and the final drying may take place in the atmosphere and, if desired, during shipment. 95

Instead of applying the sealing material by immersion, this operation may be performed by placing the lumber on a conveyor and running the pieces past spray nozzles which will discharge the material in sufficient amounts to insure that all parts of the lumber receive a coating. While it is generally preferable to apply the sealing material cold, in some instances it may be desirable to maintain the liquid at a temperature 100 above normal atmospheric. Similarly, for most purposes drying without artificial heat will be at a rate sufficiently rapid to be satisfactory, but if desired, the drying may be 105 accelerated either by heat or by fans. The details of the steps for carrying out the process will, to a large extent, depend on local conditions and on the type of wood which is undergoing treatment. 110

The sealing material which I have described as suitable for use in my process forms a clear film and is thus satisfactory for general use, but in some instances, where 115 it is known in advance that the wood is to be given a finish of a certain color, a suitable coloring material may be incorporated in the sealing solution which then acts as a vehicle. 120

Since the sealing material is used only in 125 small quantities and it is applied by a simple 130

dipping operation, as distinguished from impregnation processes heretofore used and involving impregnation under reduced pressure, the cost of the finished product is relatively low. The equipment necessary for carrying out the process is relatively inexpensive and due to the superior quality of the treated dressed lumber and its increased utility, in that it retains its dimensions and form and likewise carries a priming coat, this treated lumber may be sold at a price increase much more than sufficient to cover the increase in production cost.

I have found that the treatment according to my invention is suitable for many different kinds of wood and is particularly satisfactory with gum, pine, and oak. Gum is a wood which absorbs and gives off moisture with great rapidity, so that its use is accompanied by many difficulties, due to change in moisture content. The application of the sealing material in accordance with my invention overcomes these difficulties and makes it possible to use this wood for many purposes for which it has hitherto been considered entirely unsatisfactory. This is due to the fact that the coating applied to the lumber in accordance with the invention covers its entire exterior surface with a substantially impervious film and is applied to the lumber immediately after the dressing operations have been completed, as the result of which the lumber retains substantially unchanged that content of moisture which it possesses at the time of applying the coating, and warping, checking, etc., which occur as a consequence of changes in moisture content in the dressed lumber as now made and distributed, are substantially eliminated.

I claim:

1. A method of producing dressed lumber substantially free from defects due to change in moisture content, which comprises dressing rough dimension stock to proper size and shape, and immediately applying to the dressed product a sealing material substantially free from gums and forming a thin, hard substantially water-proof envelope on all surfaces of the wood.
2. A method of producing dressed lumber substantially free from defects due to change in moisture content, which comprises drying rough dimension stock to a selected moisture content, dressing the stock to the desired pattern, and immediately after the dressing operation is completed, applying to the dressed product a sealing material substantially free from gums and forming a thin, hard substantially water-proof envelope on all surfaces of the lumber.
3. A method of producing dressed lumber substantially free from defects due to change in moisture content, which comprises kiln-drying rough dimension stock to a selected moisture content, dressing the dried stock to the desired pattern, and applying to the dried stock a thin, substantially waterproof film, substantially free from gums, the operations of dressing the lumber and applying the film thereto being carried on without substantial delay to avoid variation in the moisture content of the lumber from that present upon completion of the drying operation.
4. A method of producing lumber substantially free from defects due to change in moisture content, which comprises drying the lumber to a selected moisture content, and immediately applying to all surfaces of the lumber a sealing material substantially free from gums which penetrates the wood to a substantial extent and also forms a thin, clear, substantially waterproof surface film having a slight sheen.
5. A method of producing lumber, which comprises drying the lumber to a selected moisture content, and applying to all surfaces of the dried lumber a mixture consisting of a water-proofing material and a volatile liquid hydrocarbon of high penetrating quality, this mixture being substantially free from gums.
6. A method of producing lumber, which comprises drying the lumber to a selected moisture content and applying to all surfaces of the dried lumber a mixture consisting of a waterproofing material which dries hard and clear and a liquid hydrocarbon which penetrates wood rapidly and dries quickly, this mixture being substantially free from gums.
7. A method of producing lumber, which comprises drying the lumber to a selected moisture content, and applying to the dried lumber a mixture consisting of China wood oil treated to give it waterproofing qualities and a liquid hydrocarbon.
8. A method of producing lumber, which comprises drying the lumber to a selected moisture content, and applying to the dried lumber a mixture consisting of China wood oil treated to give it waterproofing qualities and xylol.
9. A method of producing lumber, which comprises drying the lumber to a selected moisture content, and applying to the dried lumber a mixture consisting of China wood oil treated to give it waterproofing qualities and xylol, to which has been added a quantity of a pigment.
10. A method of producing lumber, which comprises drying the lumber to a selected moisture content, and applying to the dried lumber a mixture consisting of China wood oil treated to give it waterproofing qualities and xylol in approximately equal amounts.
11. A method of treating lumber which comprises drying the lumber to a moisture content approximating 8 per cent and coating the dried lumber with a mixture consisting of

China wood oil treated to give it waterproofing qualities and a liquid hydrocarbon.

12. A method of treating lumber, which comprises drying the lumber to a selected moisture content, immersing the dried lumber in a sealing compound consisting of a waterproofing material and a liquid of high penetrating qualities, the mixture being substantially free from gums.

10. In testimony whereof I affix my signature.  
DE VERE DIERKS.

15

20

25

30

35

40

45

50

55

60

65